

## UNITED STATES PATENT OFFICE.

JOHN W. FRAZIER, OF SAN ANTONIO, TEXAS, ASSIGNOR TO UVALDE ROCK ASPHALT COMPANY, OF SAN ANTONIO, TEXAS.

## PROCESS OF TREATING ROCK ASPHALT FOR SHIPMENT AND LAYING.

No Drawing.

Application filed August 29, 1924. Serial No. 735,021

My invention relates to a new and improved process for the preparation and shipment of limestone rock asphalt, for use in surfacing roads, streets, floors, etc.

5 Limestone rock asphalt or "rock asphalt" occurs in nature and is found in scattered deposits in different parts of the world. It comprises a pure limestone base of a porous, fossiliferous character, mostly shell, more or 10 less thoroughly and intimately impregnated with asphalt. The asphalt in this rock is approximately pure and, due to the porous character of the limestone, the lighter distillates of the bitumen have passed off in the 15 ages since its formation, leaving a hard bitumen. The said rock asphalt, as it is found in the United States, is particularly adapted to withstand wear of traffic and weather conditions when properly prepared and in- 20 stalled in place.

In consideration of my invention, it must be recognized that limestone rock asphalt is a natural product and differs widely in physical analysis from an artificial asphalt paving material or a sandstone rock asphalt, which have approximately the same chemical analysis. This difference between the limestone rock asphalt and the artificial paving material or the sandstone rock asphalt is 25 clearly indicated in the fact that the asphalt is contained within each particle in the former material, and is a coating on the outside of each particle in the two latter materials.

30 In the construction of asphalt pavements or surfacing, it has been found advisable to so govern the penetration of the asphaltic content by means of fluxing or hardening agents, that the finished product falls within 35 certain specified limits calculated to enable the material to provide satisfactory service within the range of the temperature extremes contemplated during the life of the pavement. In the construction of pavements or surfacing with limestone rock asphalt, it has been found that the material may be installed either hot or cold, but with either process, it is necessary to introduce a fluxing agent to increase the penetration of 40 the asphalt content, so as to soften the asphalt and thereby prevent cracking, as the natural state of the asphalt is too hard, and brittle to perform satisfactory service unless softened with oil. In ordinary practice it 45 has been the custom to ship the limestone

rock asphalt to the plant where it is to be prepared, in the form of rubble, spall or "one man rock".

This has been found necessary for the reason that the material, if shipped from the 50 rock asphalt mines in a finely pulverized state, would amalgamate and adhere into one mass, making the handling of the same very difficult and necessitating that it be repulverized at the point of use. After arrival at the plant, the rock asphalt is usually run through a pulverized and then into suitable mixing machines where the flux oil is added, and heat applied in case the material is to be laid hot. This method requires that 55 the plant used in preparation of the material be transported to and from each job; also workmen skilled in the operation of the plant must be transported to the location and maintained during the period of the work. 60

It is further necessary to provide power, water and storage space for each set-up, all of which adds fixed and contingent expense. The cost of transporting, setting-up and operating the necessary plant oftentimes pre- 65 cludes the use of this type of material for certain work, particularly the smaller jobs. 70

75 It is an object of my invention to provide a process by means of which the limestone rock asphalt may be prepared at the mines where it is produced, or at any other suitable location, in a manner that will permit of shipment to distant points and in a condition in which it may be readily removed 80 from the cars and be ready to lay, thus eliminating the necessity of an individual plant 85 for each job.

To accomplish this purpose, I use in addition to the limestone rock asphalt, an asphaltic base oil or other fluxing agent, 90 naphtha, and a peculiar porous limestone found in the locality of the rock asphalt mines. 95

In preparing the material, a mixing machine of ordinary construction is employed 100 and I first introduce into the mixer approximately 25% of the porous limestone, which has been previously pulverized to the desired degree of fineness. This percentage of limestone may be increased or decreased as 105 desired, and is governed to a great extent by the percentage of bitumen in the rock asphalt to be used. Next, I introduce the naphtha or other suitable solvent in an amount of approximately two to four gal- 110

2

lons to each ton of finished material and cause this to be thoroughly mixed with the limestone dust. The naptha is rapidly absorbed by the limestone in the same manner that a sponge absorbs water. The amount of naptha to be used may be varied as desired depending on the length of time the material is to be kept before laying. Next, I introduce the asphaltic oil or other fluxing agent into the mixture in sufficient quantity to provide the desired penetration in the finished product, generally about three to six gallons for each ton of finished material. Finally, I introduce the rock asphalt which has been previously pulverized to the proper fineness and cause the entire charge to be thoroughly mixed. By using this sequence, I find I obtain a perfect mixture of the ingredients in the shortest time, because the action of the naptha which has been introduced into the limestone partly dissolves the flux oil and assists in uniform distribution. Then also, it is found that the assimilation of both the naptha and the flux oil is more perfect in the limestone than it is in the rock asphalt, and that, when the pulverized rock asphalt is finally introduced, there are no accumulations, pockets or balls of the heavy fluxing oil to be broken up. However, I do not confine myself to the exact procedure or sequence described but may change at will one or more of the ingredients and the percentage used. As an illustration, it might prove advisable at certain times to use sand instead of the porous limestone, or to eliminate the limestone or sand entirely, as in the case of exceptionally lean rock asphalt.

The material thus prepared may be transported great distances, as the naptha in slowly evaporating, throws off a vapor which prevents the mixture from "setting up" or hardening, and where the porous limestone is used, this action is retarded and prolonged, permitting the material to be kept indefinitely. Also, the action of the porous limestone dust, or sand where used, tends to keep the particles of rock asphalt from coming in contact and prevents adhesion. Yet, when the material is ready for compression, a permanent bond is readily made on account of the excess amount of the rock asphalt.

When thus prepared and transported to the place where it is to be used, the material may be readily removed from the cars and hauled to the job, where it may be raked, levelled and rolled on the prepared base, which may or may not be previously treated with oil. Where desired the material may be heated before placing and rolling, but this not necessary to secure good results.

Having thus described my invention, what I claim as new and desire to protect by Letters Patent is:

1. A process of preparing limestone rock asphalt in condition for shipment ready to lay, comprising first, crushing and pulverizing a quantity of porous limestone, then mixing with said limestone a small quantity of solvent; then introducing a small proportion of fluxing agent, finely crushing limestone rock asphalt and mixing it with the prepared limestone in the proportion of about four parts of the rock asphalt to one of the prepared limestone dust.

2. A process of preparing rock asphalt for shipment ready to lay, comprising finely crushing the rock asphalt, and mixing therewith about one-fourth of its bulk in porous limestone dust treated by first mixing therewith a solvent and then a small proportion of fluxing agent in the proportion of approximately three to six gallons of flux to the ton of the charge.

3. The process of preparing rock asphalt for shipment ready to lay, including pulverizing the rock asphalt and mixing therewith a substantial proportion of porous limestone dust prepared by mixing therewith a volatile solvent, and a small quantity of asphaltic oil.

4. The process of preparing limestone rock asphalt for shipment ready to lay, comprising pulverizing the rock asphalt and mixing therewith approximately 25% of its bulk in porous limestone dust prepared by mixing therewith approximately three gallons of solvent to the ton of the total charge, and five gallons of asphaltic flux to the ton finished material.

In testimony whereof I hereunto affix my signature this 26th day of August, A. D., 1924.

JOHN W. FRAZIER.